



US006214133B1

(12) **United States Patent**  
Deevi et al.

(10) **Patent No.:** US 6,214,133 B1  
(45) **Date of Patent:** Apr. 10, 2001

(54) **TWO PHASE TITANIUM ALUMINIDE ALLOY**

(75) Inventors: **Seetharama C. Deevi**, Midlothian, VA (US); **C. T. Liu**, Oak Ridge, TN (US)

(73) Assignee: **Chrysalis Technologies, Incorporated**, Richmond, VA (US)

(\*) Notice: Subject to any disclaimer, the term of this patent is extended or adjusted under 35 U.S.C. 154(b) by 0 days.

(21) Appl. No.: **09/174,103**

(22) Filed: **Oct. 16, 1998**

(51) Int. Cl.<sup>7</sup> ..... **C22C 14/00**

(52) U.S. Cl. ..... **148/421**; 420/418

(58) Field of Search ..... 148/421; 420/418

(56) **References Cited**

U.S. PATENT DOCUMENTS

|           |        |               |         |
|-----------|--------|---------------|---------|
| 4,842,819 | 6/1989 | Huang et al.  | 420/418 |
| 4,917,858 | 4/1990 | Eylon et al.  | 419/28  |
| 5,196,162 | 3/1993 | Maki et al.   | 420/418 |
| 5,232,661 | 8/1993 | Matsuo et al. | 420/421 |
| 5,342,577 | 8/1994 | Nazmy et al.  | 420/418 |
| 5,348,702 | 9/1994 | Matsuo et al. | 420/421 |

|           |         |                     |         |
|-----------|---------|---------------------|---------|
| 5,350,466 | 9/1994  | Larsen, Jr. et al.  | 148/421 |
| 5,370,839 | 12/1994 | Masahashi et al.    | 420/418 |
| 5,417,781 | 5/1995  | McQuay et al.       | 148/671 |
| 5,429,796 | 7/1995  | Larsen, Jr.         | 420/590 |
| 5,489,411 | 2/1996  | Jha et al.          | 419/3   |
| 5,503,794 | 4/1996  | Ritter et al.       | 419/28  |
| 5,530,225 | 6/1996  | Hajaligol           | 219/535 |
| 5,591,368 | 1/1997  | Fleischhauer et al. | 219/535 |
| 5,634,992 | 6/1997  | Kelly et al.        | 148/669 |
| 5,746,846 | 5/1998  | Kim et al.          | 148/671 |

Primary Examiner—John Sheehan

(74) Attorney, Agent, or Firm—Burns, Doane, Swecker & Mathis, LLP

(57) **ABSTRACT**

A two-phase titanic aluminide alloy having a lamellar microstructure with little intercolony structures. The alloy can include fine particles such as boride particles at colony boundaries and/or grain boundary equiaxed structures. The alloy can include alloying additions such as  $\leq 10$  at % W, Nb and/or Mo. The alloy can be free of Cr, V, Mn, Cu and/or Ni and can include, in atomic %, 45 to 55% Ti, 40 to 50% Al, 1 to 5% Nb, 0.3 to 2% W, up to 1% Mo and 0.1 to 0.3% B. In weight %, the alloy can include 57 to 60% Ti, 30 to 32% Al, 4 to 9% Nb, up to 2% Mo, 2 to 8% W and 0.02 to 0.08% B.

19 Claims, 17 Drawing Sheets





**FIG. 1A**



**FIG. 1B**



**FIG. 1C**



**FIG. 1D**



**FIG.2A**



**FIG.2B**



**FIG.2C**



**FIG.2D**



**FIG.3**



**FIG.4**



**FIG.5A**



**FIG.5B**



**FIG.6A**



**FIG.6B**



**FIG.7A**



**FIG.7B**



**FIG.8A**



**FIG.8B**



**FIG. 9A**



**FIG. 9B**



**FIG.10**



**FIG. 11A**



**FIG. 11B**



**FIG.11C**



**FIG.11D**



FIG.12



FIG.13



FIG.14



FIG.15



FIG. 16

## TWO PHASE TITANIUM ALUMINIDE ALLOY

### STATEMENT OF GOVERNMENT RIGHTS

The United States government has rights in this invention pursuant to contract No. DE-AC05-84OR21400 between the United States Department of Energy and Lockheed Martin Energy Research Corporation, Inc.

### FIELD OF THE INVENTION

The invention relates generally to two-phase titanium aluminide alloy compositions useful for resistive heating and other applications such as structural applications.

### BACKGROUND OF THE INVENTION

Titanium aluminide alloys are the subject of numerous patents and publications including U.S. Pat. Nos. 4,842,819; 4,917,858; 5,232,661; 5,348,702; 5,350,466; 5,370,839; 5,429,796; 5,503,794; 5,634,992; and 5,746,846, Japanese Patent Publication Nos. 63-171862; 1-259139; and 142539; European Patent Publication No. 365174 and articles by V. R. Ryabov et al entitled "Properties of the Intermetallic Compounds of the System Iron-Alminum" published in Metal Metalloved, 27, No.4, 668673, 1969; S. M. Barinov et al entitled "Deformation and Failure in Titanium Aluminide" published in Izvestiya Akademii Nauk SSSR Metally, No. 3, 164-168, 1984; W. Wunderlich et al entitled "Enhanced Plasticity by Deformation Twinning of Ti-Al-Base Alloys with Cr and S" published in Z. Metallkunde, 802-808, 11/1990; T. Tsujimoto entitled "Research, Development, and Prospects of TiAl Intermetallic Compound Alloys" published in Titanium and Zirconium, Vol. 33, No. 3, 19 pages, 7/1985; N. Maeda entitled "High Temperature Plasticity of Intermetallic Compound TiAl" presented at Material of 53<sup>rd</sup> Meeting of Superplasticity, 13 pages, 1/30/1990; N. Maeda et al entitled "Improvement in Ductility of Intermetallic Compound through Grain Super-refinement" presented at Autumn Symposium of the Japan Institute of Metals, 14 pages, 1989; S. Noda et al entitled "Mechanical Properties of TiAl Intermetallic Compound" presented at Autumn Symposium of the Japan Institute of Metals, 3 pages, 1988; H. A. Lipsitt entitled "Titanium Aluminides—An Overview" published in Mat. Res. Soc. Symp. Proc. Vol. 39, 351-364, 1985; P. L. Martin et al entitled "The Effects of Alloying on the Microstructure and Properties of Ti<sub>3</sub> Al and TiAl" published by ASM in Titanium 80, Vol. 2, 1245-1254, 1980; S. H. Whang et al entitled "Effect of Rapid Solidification in L<sub>1</sub><sub>0</sub> TiAl Compound Alloys" ASM Symposium Proceedings on Enhanced Properties in Structural Metals Via Rapid Solidification, Materials Week, 7 pages, 1986; and D. Vujic et al entitled "Effect of Rapid Solidification and Alloying Addition on Lattice Distortion and Atomic Ordering in L<sub>1</sub><sub>0</sub> TiAl Alloys and Their Ternary Alloys" published in Metallurgical Transactions A, Vol. 19A, 2445-2455, 10/1988.

Methods by which TiAl aluminides can be processed to achieve desirable properties are disclosed in numerous patents and publications such as those mentioned above. In addition, U.S. Pat. No. 5,489,411 discloses a powder metallurgical technique for preparing titanium aluminide foil by plasma spraying a coatable strip, heat treating the strip to relieve residual stresses, placing the rough sides of two such strips together and squeezing the strips together between pressure bonding rolls, followed by solution annealing, cold rolling and intermediate anneals. U.S. Pat. No. 4,917,858 discloses a powder metallurgical technique for making tita-

nium aluminide foil using elemental titanium, aluminum and other alloying elements. U.S. Pat. No. 5,634,992 discloses a method of processing a gamma titanium aluminide by consolidating a casting and heat treating the consolidated casting above the eutectoid to form gamma grains plus lamellar colonies of alpha and gamma phase, heat treating below the eutectoid to grow gamma grains within the colony structure and heat treating below the alpha tansus to reform any remaining colony structure a structure having % laths within gamma grains.

Still, in view of the extensive efforts to improve properties of titanium aluminides, there is a need for improved alloy compositions and economical processing routes.

According to a first embodiment, the invention provides a two-phase titanium aluminum alloy having a lamellar microstructure controlled by colony size. The alloy can be provided in various forms such as in the as-cast, hot extruded, cold and hot worked, or heat treated condition. As an end product, the alloy can be fabricated into an electrical resistance heating element having a resistivity of 60 to 200  $\mu\Omega\text{-cm}$ . The alloy can include additional elements which provide fine particles such as second-phase or boride particles at colony boundaries. The alloy can include grain-boundary equiaxed structures. The additional alloying elements can include, for example, up to 10 at % W, Nb and/or Mo. The alloy can be processed into a thin sheet having a yield strength of more than 80 ksi (560 MPa), an ultimate tensile strength of more than 90 ksi (630 MPa), and/or tensile elongation of at least 1.5%. The aluminum can be present in an amount of 40 to 50 at %, preferably about 46 at %. The titanium can be present in the amount of at least 45 at %, preferably at least 50 at %. As an example, the alloy can include 45 to 55 at % Ti, 40 to 50 at % Al, 1 to 5 at % Nb, 0.5 to 2 at % W, and 0.1 to 0.3 at % B. The alloy is preferably free of Cr, V, Mn and/or Ni.

### BRIEF DESCRIPTION OF THE DRAWINGS

FIGS. 1a-d are optical micrographs at 200 $\times$  of PMTA TiAl alloys hot extruded at 1400° C. and annealed for 2 hours at 1000° C. FIG. 1a shows the microstructure of PMTA-1, FIG. 1b shows the microstructure of PMTA-2, FIG. 1c shows the microstructure of PMTA-3 and FIG. 1d shows the microstructure of PMTA4;

FIGS. 2a-d show optical micrographs at 500 $\times$  of PMTA alloys hot extruded at 1400° C. and annealed for 2 hours at 1000° C. FIG. 2a shows the microstructure of PMTA-1, FIG. 2b shows the microstructure of PMAT-2, FIG. 2c shows the microstructure of PMAT-3 and FIG. 2d shows the microstructure of PMTA4;

FIG. 3 shows ghost-pattern bands observed in a back-scattered image of PMTA-2 hot extruded at 1400° C. and annealed for 2 hours at 1000° C. wherein the non-uniform distribution of W is shown;

FIG. 4 shows a back-scattered image of PMTA-2 hot extruded at 1400° C. and annealed for 2 hours at 1000° C.;

FIG. 5a is a micrograph at 200 $\times$  of PMTA-3 hot extruded at 1400° C and annealed for one day at 1000° C. and FIG. 5b shows the same microstructure at 500 $\times$ ;

FIG. 6a shows the microstructure at 200 $\times$  of PMTA-2 hot extruded at 1400° C. and annealed for 3 days at 1000° C. and FIG. 6b shows the same microstructure at 500 $\times$ ;

FIG. 7a is an optical micrograph of TiAl sheet (Ti45Al-5Cr, at %) in the as-received condition and FIG. 7b shows the same microstructure after annealing for 3 days at 1000° C., both micrographs at 500 $\times$ ;

FIG. 8a shows a micrograph of PMTA-6 and FIG. 8b shows a micrograph of PMTA-7, both of which were hot extruded at 1380° C. (magnification 200 x);

FIG. 9a is a micrograph of PMTAL and FIG. 9b is a micrograph of PMTA-7, both of which were hot extruded at 1365° C. (magnification 200 x);

FIG. 10 is micrograph showing abnormal grain growth in PMTA hot extruded at 1380° C.;

FIGS. 11a-d are micrographs of PMTA-8 heat treated at different conditions after hot extrusion at 1335° C., the heat treatments being two hours at 1000° C. for FIG. 11a, 30 minutes at 1340° C. for FIG. 11b, 30 minutes at 1320° C. for FIG. 11c, and 30 minutes at 1315° C. for FIG. 11d (magnification 200 x);

FIG. 12 is a graph of resistivity in microhms versus temperature for samples 1 and 2 cut from an ingot having a PMTA4 nominal composition;

FIG. 13 is a graph of hemispherical total emissivity versus temperature for samples 1 and 2;

FIG. 14 is a graph of diffusivity versus temperature for samples 80259-1, 80259-2 and 80259-3 cut from the same ingot as samples 1 and 2;

FIG. 15 is a graph of specific heat versus temperature for titanium aluminide in accordance with the invention; and

FIG. 16 is a graph of thermal expansion versus temperature for samples 80259-1H, 80259-1C, 80259-2H, 80259-3H, and 80259-3C cut from the same ingot as samples 1 and 2.

#### DETAILED DESCRIPTION OF THE PREFERRED EMBODIMENTS

The invention provides two-phase TiAl alloys with thermo-physical and mechanical properties useful for various applications such as resistance heater elements. The alloys exhibit useful mechanical properties and corrosion resistance at elevated temperatures up to 1000° C. and above. The TiAl alloys have extremely low material density (about 4.0 g/cm<sup>3</sup>), a desirable combination of tensile ductility and strength at room and elevated temperatures, high electrical resistance, and/or can be fabricated into sheet material with thickness <10 mil. One use of such sheet material is for resistive heating elements of devices such as cigarette lighters. For instance, the sheet can be formed into a tubular heating element having a series of heating strips which are individually powered for lighting portions of a cigarette in an electrical smoking device of the type disclosed in U.S. Pat. Nos. 5,591,368 and 5,530,225, the disclosures of which are hereby incorporated by reference. In addition, the alloys can be free of elements such as Cr, V, Mn and/or Ni.

Compared to TiAl alloys containing 1 to 4 at % Cr, V, and/or Mn for improving tensile ductility at ambient temperatures, according to the present invention, tensile ductility of dual-phase TiAl alloys with lamellar structures can be mainly controlled by colony size, rather than such alloying elements. The invention thus provides high strength TiAl alloys which can be free of Cr, V, Mn and/or Ni.

Table 1 lists nominal compositions of alloys investigated wherein the base alloy contains 46.5 at % Al, balance Ti. Small amounts of alloying additions were added for investigating effects on mechanical and metallurgical properties of the twophase TiAl alloys. Nb in amounts up to 4% was examined for possible effects on oxidation resistance, W in amounts of up to 1.0% was examined for effects on microstructural stability and creep resistance, and Mo in amounts

of up to 0.5% was examined for effects on hot fabrication. Boron in amounts up to 0.18% was added for refinement of lamellar structures in the dual-phase TiAl alloys.

Eight alloys identified as PMTA-1 to 9, having the compositions listed in Table 1, were prepared by arc melting and drop casting into a 1" diameter×5" long copper mold, using commercially-pure metals. All the alloys were successfully cast without casting defects. Seven alloy ingots (PMTA-1 to 4 and 6 to 9) were then canned in Mo cans and hot extruded at 1335 to 1400° C. with an extrusion ratio of 5:1 to 6:1. The extrusion conditions are listed in Table 2. The cooling rate after extrusion was controlled by air cooling and quenching the extruded rods in water for a short time. The alloy rods extruded at 1365 to 1400° C. showed an irregular shape whereas PMTA-8 hotextruded at 1335° C. exhibited much smoother surfaces without surface irregularities. However, no cracks were observed in any of the hot-extruded alloy rods.

The microstructures of the alloys were examined in the as-cast and heat treated conditions (listed in Table 2) by optical metallography and electron superprobe analyses. In the as-cast condition, all the alloys showed lamellar structure with some degree of segregation and coring. FIGS. 1 and 2 show the optical micrographs, with a magnification of 200 x and 500 x, respectively, for hot extruded alloys PMTA-1 to 4 stress-relieved for 2 hours at 1000° C. All the alloys showed fully lamellar structures, with a small amount of equiaxed grain structures at colony boundaries. Some fine particles were observed at colony boundaries, which are identified as borides by electron microprobe analyses. Also, there is no apparent difference in microstructural features among these four PMTA alloys.

Electron microprobe analyses reveal that tungsten is not uniformly distributed even in the hot extruded alloys. As shown in FIG. 3, the ghost-pattern bands in a darker contrast are found to be depleted with about 0.33 at % W. FIG. 4 is a back-scattered image of PMTA-2, showing the formation of second-phase particles (borides) in a bright contrast at colony boundaries. The composition of the borides was determined and listed in Table 3 together with that of the lamellar matrix. The second-phase particles are essentially (Ti,W,Nb) borides, which are decorated and pinned lamellar colony boundaries.

FIGS. 5 and 6 show the optical microstructures of hot extruded PMTA-3 and 2 annealed for 1 day and 3 days at 1000° C., respectively. Grain-boundary equiaxed structures are clearly observed in these long-term annealed specimens, and the amount increases with the annealing time at 1000° C. A significant amount of equiaxed grain structures exists in the specimen annealed for 3 days at 1000° C.

For comparison purposes, a 9-mil thick TiAl sheet (Ti45Al-5Cr, at %) was evaluated. FIG. 7 shows the optical microstructures of the TiAlCr sheet in both as-received and annealed (3 days at 1000° C.) conditions. In contrast to the dual-phase lamellar structure of the alloys according to the invention, the TiAlCr sheet has a duplex structure, and its grain structure shows no significant coarsening at 1000° C.

Tensile sheet specimens with a thickness of 9–20 mils and a gage length of 0.5 in were sectioned from the hot extruded alloys rods after annealing for 2 hours at 1000° C., using a EDM machine. Some of the specimens were re-annealed up to 3 days at 1000° C. prior to tensile testing. Tensile tests were performed on an Instron testing machine at a strain rate of 0.1 inch/second at room temperature. Table 4 summarizes the tensile test results.

All the alloys stress-relieved for 2 hours at 1000° C. exhibited 1% or more tensile elongation at room temperature

in air. The tensile elongation was not affected when the specimen thickness varied from 9 to 20 mils. As indicated in Table 4, among the 4 alloys, alloy PMTAA appears to have the best tensile ductility. It should be noted that a tensile elongation of 1.6% obtained from a 20-mil thick sheet specimen is equivalent to 4% elongation obtained from rod specimens with a gage diameter of 0.12 in. The tensile elongation appears to increase somewhat with annealing time at 1000° C., and the maximum ductility is obtained in the specimen annealed for 1 day at 1000° C.

All the alloys are exceptionally strong, with a yield strength of more than 100 ksi (700 MPa) and ultimate tensile strength more than 115 ksi (800 MPa) at room temperature. The high strength is due to the refined fully lamellar structures produced in these TiAl alloys. In comparison, the TiAlCr sheet material has a yield strength of only 61 ksi (420 MPa) at room temperature. Thus, the PMTA alloys are stronger than the TiAlCr sheet by as much as 67%. The PMTA alloys including 0.5% Mo exhibited significantly increased strengths, but slightly lower tensile elongation at room temperature.

FIGS. 8a-b and 9a-b show the optical micrographs of PMTA6 and 7 hot extruded at 1380° C. and 1365° C., respectively. Both alloys showed lamellar grain structures with little intercolony structures. Large colony grains (see FIG. 10) were observed in both alloys hot extruded at 1380° C. and 1365° C., which probably resulted from abnormal grain growth in the alloys containing low levels of boron after hot extrusion. There is no significant difference in microstructural features in these two PMTA alloys.

FIGS. 11a-d show the effect of heat treatment on microstructures of PMTA-8 hot extruded at 1335° C. The alloy extruded at 1335° C. showed much fewer colony size and much more intercolony structures, as compared with those hot extruded at 1380° C. and 1365° C. Heat treatment for 2 h at 1000° C. did not produce any significant change in the as-extruded structure (FIG. 11a). However, heat treatment for 30 mins at 1340° C. resulted in a substantially larger colony structure (FIG. 11b). Lowering the heat-treatment temperature from 1340° C. to 1320-1315° C. (a difference by 20-25° C.) produced a sharp decrease in colony size, as indicated by FIGS. 11c and 11d. The annealing at 1320-1315° C. also appears to produce more intercolony structures in PMTA-8. The abnormal grain growth is almost completely eliminated by hot extrusion at 1335° C.

Tensile sheet specimens of PMTA-6 to 8 with a thickness varying from 8 to 22 mils and with a gage length of 0.5 inch were sectioned from the hot extruded alloy rods after giving a final heat treatment of 2 h at 1000° C. or 20 min at 1320-1315° C., using an EDM machine. Tensile tests were performed on an Instron testing machine at a strain rate of 0.1 in/s at temperatures up to 800° C. in air. All tensile results are listed in Tables 5 to 8. The alloys PMTA4, -6 and -7 heat treated for 2 h at 1000° C. showed excellent strengths at all temperatures, independent of hot extrusion temperature. The hot extrusion at 1400-1365° C. gives low tensile ductilities (<4%) at room and elevated temperatures. A significant increase in tensile ductility is obtained at all temperatures when hot extruded at 1335° C. PMTA-8 which was hot extruded at 1335° C. exhibited the highest strength and tensile ductility at all test temperatures. There did not appear to be any systematical variation of tensile ductility with specimen thickness varying from 8 to 22 mils.

Tables 7 and 8 also show the tensile properties of PMTA-6 and 7 heat treated for 20 min. at 1320° C. and 1315° C., respectively. As compared with the results obtained from

heat treatment at 1000° C., the heat treatment at 1320-1315° C. resulted in higher tensile elongation, but lower strength at the test temperatures. Among all the alloys and heat treatments, PMTA-8 hot extruded at 1335° C. and annealed for 20 min at 1315° C. exhibited the best tensile ductility at room and elevated temperatures. This alloy showed a tensile ductility of 3.3% and 11.7% at room temperature and 800° C., respectively. PMTA-8 heat treated at 1315° C. appears to be substantially stronger than known TiAl alloys.

In an attempt to demonstrate the bend ductility of TiAl sheet material, several pieces of 11 to 20 mil PMTA-7 and PMTA-8 alloy sheets, produced by hot extrusion and heat treated at 1320° C., were bent at room temperature. Each alloy piece did not fracture after a bend of 42°. These results clearly indicate that PMTA alloys with a controlled microstructure is bendable at room temperature.

The oxidation behavior of PMTA-2, -5 and -7 was studied by exposing sheet samples (9-20 mils thick) at 800° C. in air. The samples were periodically removed from furnaces for weight measurement and surface examination. The samples showed a very low weight gain without any indication of spalling. It appears that the alloying additions of W and Nb affect the oxidation rate of the alloys at 800° C., and W is more effective in improving the oxidation resistance of TiAl alloys. Among the alloys, PMTA-7 exhibits the lowest weight gain and the best oxidation resistance at 800° C. Oxidation of PMTA-7 indicated that oxide scales are fully adherent with no indication of microcracking and spalling. This observation clearly suggests that the oxide scales formed at 800° C. are well adherent to the base material and are very protective.

FIG. 12 is a graph of resistivity in microhms versus temperature for samples 1 and 2 which were cut from an ingot having a nominal composition of PMTA4, i.e. 30.8 wt % Al, 7.1 wt % Nb, 2.4 wt % W, and 0.045 wt % B.; FIG. 13 is a graph of hemispherical total emissivity versus temperature for samples 1 and 2; FIG. 14 is a graph of diffusivity versus temperature for samples 80259-1, 80259-2 and 80259-3 cut from the same ingot as samples 1 and 2; FIG. 15 is a graph of specific heat versus temperature for titanium aluminide in accordance with the invention; and FIG. 16 is a graph of thermal expansion versus temperature for samples 80259-1H, 80259-1C, 80259-2H, 80259-3H, and 80259-3C cut from the same ingot as samples 1 and 2.

In summary, the hot PMTA alloys extruded at 1365 to 1400° C. exhibited mainly lamellar structures with little intercolony structures while PMTA-8 extruded at 1335° C. showed much finer colony structures and more intercolony structures. The heat treatment of PMTA-8 at 1315-1320° C. for 20 min. resulted in fine lamellar structures. The alloys may include (Ti,W,Nb) borides formed at colony boundaries. Moreover, tungsten in the hot-extruded alloys is not uniformly distributed, suggesting the possibility of high electrical resistance of TiAl alloys containing W additions. The inclusion of 0.5 at. % Mo significantly increases the yield and ultimate tensile strengths of the TiAl alloys, but lowers the tensile elongation to a certain extent at room temperature. Among the four hot extruded alloys PMTA 14, PMTA4 with the alloy composition Ti-46.5 Al-3 Nb-0.5 W-0.2 B (at %) has the best combination of tensile ductility and strength at room temperature. In comparison with the TiAlCr sheet material (Ti45 Al-5Cr), PMTA4 is stronger than the TiAlCr sheet by 67%. In addition, the TiAlCr sheet showed no bend ductility at room temperature while PMTAA has an elongation of 1.4%. The tensile elongation of TiAl alloys is independent of sheet thickness in the range of 9 to 20 mils. The alloys PMTA 4, 6 and 7 heat treated at

1000° C. for 2 h showed excellent strength at all temperatures up to 800° C., independent of hot extrusion temperature. Hot extrusion temperatures of 1400–1365° C., however, provides lower tensile ductilities (<4%) at room and elevated temperatures. A significant increase in tensile ductility is obtained at all temperatures when the extrusion temperature is 1335° C. PMTA-8 (Ti46.5 Al-3 Nb-1W-0.5B) hot extruded at 1335° C. and annealed at 1315° C. for 20 min. exhibited the best tensile ductility at room and elevated temperatures (3.3% at room temperature and 11.7% at 800° C.).

TABLE 1

| Alloy number        | Nominal Alloy Compositions |      |    |    |     |     |      |
|---------------------|----------------------------|------|----|----|-----|-----|------|
|                     | Ti                         | Al   | Cr | Nb | Mo  | W   | B    |
| Compositions (at %) |                            |      |    |    |     |     |      |
| Compositions (wt %) |                            |      |    |    |     |     |      |
| PMTA-1              | 50.35                      | 46.5 | 0  | 2  | 0.5 | 0.5 | 0.15 |
| PMTA-2              | 50.35                      | 46.5 | 0  | 2  | —   | 1.0 | 0.15 |
| PMTA-3              | 49.85                      | 46.5 | 0  | 2  | 0.5 | 1.0 | 0.15 |
| PMTA-4              | 49.85                      | 46.5 | 0  | 3  | —   | 0.5 | 0.15 |
| PMTA-5              | 47.85                      | 46.5 | 0  | 4  | —   | 0.5 | 0.15 |
| PMTA-6              | 49.92                      | 46.5 | 0  | 3  | —   | 0.5 | 0.08 |
| PMTA-7              | 49.92                      | 46.5 | 0  | 3  | —   | 1.0 | 0.08 |
| PMTA-8              | 49.40                      | 46.5 | 0  | 3  | —   | 1.0 | 0.10 |
| PMTA-9              | 49.32                      | 46.5 | 0  | 3  | —   | 1.0 | 0.18 |

TABLE 2

| Fabrication and Heat Treatment Condition Used for PMTA Alloys |                                  |                                |
|---------------------------------------------------------------|----------------------------------|--------------------------------|
| Alloy number                                                  | Hot extrusion temperature (° C.) | Heat treatment (° C./time)     |
| PMTA-1                                                        | 1400                             | 1000° C. for up to 3 days      |
| PMTA-2                                                        | 1400                             | 1000° C. for up to 3 days      |
| PMTA-3                                                        | 1400                             | 1000° C. for up to 3 days      |
| PMTA-4                                                        | 1400                             | 1000° C. for up to 3 days      |
| PMTA-5                                                        |                                  |                                |
| PMTA-6                                                        | 1380, 1365                       | 1000° C./2 hours               |
| PMTA-7                                                        | 1380, 1365                       | 1000° C./2 hr, 1320° C./20 min |
| PMTA-8                                                        | 1335                             | 1000° C./2 hr, 1315° C./20 min |

TABLE 3

| Phase Compositions in PMTA-2 Alloy Determined by Electron Microprobe Analyses |         |       |      |                       |
|-------------------------------------------------------------------------------|---------|-------|------|-----------------------|
| Phase                                                                         | Ti      | Al    | W    | Alloy elements (at %) |
|                                                                               |         |       |      | Nb                    |
| Matrix phase (dark contrast)                                                  | Balance | 44.96 | 0.82 | 1.32                  |
| Matrix phase (bright contrast)                                                | Balance | 44.70 | 1.15 | 1.32                  |
| Borides*                                                                      | 77.69   | 8.66  | 9.98 | 3.67                  |

\*metals elements only

TABLE 4

| Alloy number     | Composition<br>Nb—Mo—W<br>(at %) | Tensile Properties of PMTA Alloys<br>Hot Extruded at 1400° C. and Tested at Room Temperature |                  |                   |
|------------------|----------------------------------|----------------------------------------------------------------------------------------------|------------------|-------------------|
|                  |                                  | elongation (%)                                                                               | $\sigma_y$ (ksi) | $\rho_{ue}$ (ksi) |
| 2 hours/1000° C. |                                  |                                                                                              |                  |                   |
| PMTA-1           | 2/0/0.5                          | 1.0                                                                                          | 114              | 118               |
| PMTA-2           | 2/0/1.0                          | 1.2                                                                                          | 104              | 117               |
| PMTA-3           | 2/0/5/1.0                        | 1.1                                                                                          | 123              | 132               |
| PMTA-4           | 3/0/0.5                          | 1.4                                                                                          | 102              | 115               |
| 1 day/1000° C.   |                                  |                                                                                              |                  |                   |
| PMTA-3           | 2/0/5/1.0                        | 1.4                                                                                          | 115              | 131               |
| 3 days/1000° C.  |                                  |                                                                                              |                  |                   |
| PMTA-2           | 2/0/1.0                          | 0.8                                                                                          | 105              | 109               |

TABLE 5

| Test temperature (° C.) | Yield strength (ksi) | Ultimate tensile strength (ksi) | Elongation (%) | Tensile Properties of PMTA-4 Hot Extruded at 1400° C. and Annealed for 2 h at 1000° C. |     |
|-------------------------|----------------------|---------------------------------|----------------|----------------------------------------------------------------------------------------|-----|
|                         |                      |                                 |                | 22                                                                                     | 600 |
| 22                      | 102.0                | 115                             | 1.4            |                                                                                        |     |
| 600                     | 101.0                | 127                             | 2.4            |                                                                                        |     |
| 700                     | 96.5                 | 130                             | 2.7            |                                                                                        |     |
| 800                     | 97.8                 | 118                             | 2.4            |                                                                                        |     |

TABLE 6

| Test temperature (° C.) | Yield strength (ksi) | Ultimate tensile strength (ksi) | Elongation (%) | Tensile Properties of PMTA-6 Hot Extruded at 1365° C. and Annealed at 1000° C. for 2 h |     |
|-------------------------|----------------------|---------------------------------|----------------|----------------------------------------------------------------------------------------|-----|
|                         |                      |                                 |                | 22                                                                                     | 300 |
| 22                      | 121.0                | 136                             | 1.3            |                                                                                        |     |
| 300                     | 101.0                | 113                             | 1.2            |                                                                                        |     |
| 700                     | 93.6                 | 125                             | 2.7            |                                                                                        |     |
| 800                     | 86.5                 | 125                             | 3.9            |                                                                                        |     |

TABLE 7

| Test temperature (° C.)         | Yield strength (ksi) | Ultimate tensile strength (ksi) | Elongation (%) | Tensile Properties of PMTA-7 Hot Extruded at 1365° C. |     |
|---------------------------------|----------------------|---------------------------------|----------------|-------------------------------------------------------|-----|
|                                 |                      |                                 |                | 22                                                    | 300 |
| 22                              | 116.0                | 122                             | 1.0            |                                                       |     |
| 300                             | 101.0                | 116                             | 1.5            |                                                       |     |
| 700                             | 105.0                | 131                             | 2.7            |                                                       |     |
| 800                             | 87.2                 | 121                             | 3.1            |                                                       |     |
| Annealed for 2 h at 1000° C.    |                      |                                 |                |                                                       |     |
| 20                              | 84.5                 | 106.0                           | 3.0            |                                                       |     |
| 300                             | 71.4                 | 89.8                            | 2.5            |                                                       |     |
| 700                             | 68.5                 | 97.2                            | 4.5            |                                                       |     |
| 800                             | 63.5                 | 90.2                            | 4.5            |                                                       |     |
| Annealed for 20 min at 1320° C. |                      |                                 |                |                                                       |     |

TABLE 8

| Tensile Properties of PMTA-8 Hot Extruder at 1335° C. |                         |                                    |                   |
|-------------------------------------------------------|-------------------------|------------------------------------|-------------------|
| Test temperature<br>(° C.)                            | Yield strength<br>(ksi) | Ultimate tensile<br>strength (ksi) | Elongation<br>(%) |
| Annealed for 2 h at 1000° C.                          |                         |                                    |                   |
| 22                                                    | 122.0                   | 140                                | 2.0               |
| 300                                                   | 102.0                   | 137                                | 4.3               |
| 700                                                   | 95.0                    | 131                                | 4.7               |
| 800                                                   | 90.2                    | 124                                | 5.6               |
| Annealed for 20 min at 1315° C.                       |                         |                                    |                   |
| 20                                                    | 96.2                    | 116                                | 3.3               |
| 300                                                   | 79.4                    | 115                                | 6.1               |
| 700                                                   | 72.2                    | 112                                | 7.5               |
| 800                                                   | 72.0                    | 100                                | 11.7              |

The foregoing titanium aluminide can be manufactured into various shapes or products such as electrical resistance heating elements. However, the compositions disclosed herein can be used for other purposes such as in thermal spray applications wherein the compositions could be used as coatings having oxidation and corrosion resistance. Also, the compositions could be used as oxidation and corrosion resistant electrodes, furnace components, chemical reactors, sulfidization resistant materials, corrosion resistant materials for use in the chemical industry, pipe for conveying coal slurry or coal tar, substrate materials for catalytic converters, exhaust walls and turbocharger rotors for automotive and diesel engines, porous filters, etc.

With respect to resistance heating elements, the geometry of the heating element blades can be varied to optimize heater resistance according to the formula:  $R=\rho(L/W \times T)$  wherein  $R$ =resistance of the heater,  $\rho$ =resistivity of the heater material,  $L$ =length of heater,  $W$ =width of heater and  $T$ =thickness of heater. The resistivity of the heater material can be varied by changes in composition such as adjusting the aluminum content of the heater material, processing or by incorporation of alloying additions. For instance, the resistivity can be significantly increased by incorporating particles of alumina in the heater material. The heater material can optionally include ceramic particles to enhance creep resistance and/or thermal conductivity. For instance, the heater material can include particles or fibers of electrically conductive material such as nitrides of transition metals (Zr, Ti, Hf), carbides of transition metals, borides of transition metals and MoS<sub>2</sub> for purposes of providing good high temperature creep resistance up to 1200° C. and also excellent oxidation resistance. The heater material may also incorporate particles of electrically insulating material such as Al<sub>2</sub>O<sub>3</sub>, Y<sub>2</sub>O<sub>3</sub>, Si<sub>3</sub>N<sub>4</sub>, ZrO<sub>2</sub> for purposes of making the heater material creep resistant at high temperature and also improving thermal conductivity and/or reducing the thermal coefficient of expansion of the heater material. The electrically insulating/conductive particles/fibers can be added to a powder mixture of Fe, Al, Ti or iron aluminide or such particles/fibers can be formed by reaction synthesis of elemental powders which react exothermically during manufacture of the heater element.

The foregoing has described the principles, preferred embodiments and modes of operation of the present invention. However, the invention should not be construed as being limited to the particular embodiments discussed. Thus,

the above-described embodiments should be regarded as illustrative rather than restrictive, and it should be appreciated that variations may be made in those embodiments by workers skilled in the art without departing from the scope of the present invention as defined by the following claims.

What is claimed is:

1. A two phase Cr-free and Mu-free titanium aluminide alloy consisting essentially of, in weight %, 50 to 65% Ti, 25 to 35% Al, 2 to 15% Nb, less than 5% Mo, 1 to 10% W, and 0.01 to 0.2% B.
2. The titanium aluminide alloy of claim 1, in an as-cast, hot extruded, cold worked, or heat treated condition.
3. The titanium aluminide alloy of claim 1, wherein the alloy has a two-phase lamellar microstructure with fine particles are located at colony boundaries.
4. The titanium aluminide alloy of claim 3, wherein fine boride particles are located at the colony boundaries.
5. The titanium aluminide alloy of claim 3, wherein fine second-phase particles are located at the colony boundaries.
6. The titanium aluminide alloy of claim 1, wherein the alloy has a two-phase microstructure including grain-boundary equiaxed structures.
7. The titanium aluminide alloy of claim 1, wherein the Ti content is 57 to 60%, the Al content is 30 to 32%, the Nb content is 4 to 9%, the Mo content is at most 2%, the W content is 2 to 8% and the B content is 0.02 to 0.08%.
8. The titanium aluminide alloy of claim 1, having a yield strength of more than 80 ksi (560 MPa), an ultimate tensile strength of more than 90 ksi (680 MPa) and/or tensile elongation of at least 1%.
9. The titanium aluminide alloy of claim 1, wherein the alloy has a microstructure in which W is distributed non-uniformly.
10. The titanium aluminide alloy of claim 1, wherein aluminum is present in an amount of about 46 to 47 atomic %.
11. The titanium aluminide alloy of claim 1, wherein the alloy has a lamellar microstructure substantially free of equiaxed structures at colony boundaries.
12. The titanium aluminide alloy of claim 1, wherein the alloy does not include Mo.
13. The titanium aluminide alloy of claim 1, wherein the Ti content is 57 to 60%, the Al content is 30 to 32%, the Nb content is 4 to 9%, the W content is 2 to 8% and the B content is 0.02 to 0.08%.
14. The titanium aluminide alloy of claim 1, including 45 to 55 at % Ti, 40 to 50 at % Al, 1 to 5 at % Nb, 0.3 to 1.5 at % W, and 0.1 to 0.3 at % B.
15. The titanium aluminide alloy of claim 1, comprising a sheet with a thickness of 8 to 30 mils.
16. The titanium aluminide alloy of claim 1, free of Cr, V, Co, Cu and Ni.
17. The titanium aluminide alloy of claim 1, comprising TiAl with 2 to 4 at % Nb,  $\leq 1$  at % Mo and 0.5 to 2 at % W, 0.1 to 0.3 at % B.
18. The titanium aluminide alloy of claim 1, including 1 to 4 at % Nb,  $\leq 1$  at % Mo and 0.25 to 2 at % W.
19. The titanium aluminide alloy of claim 1, wherein the alloy has been formed into an electrical resistance heating element capable of heating to 900° C. in less than 1 second when a voltage of up to 10 volts and up to 6 amps is passed through the heating element.

\* \* \* \* \*

UNITED STATES PATENT AND TRADEMARK OFFICE  
**CERTIFICATE OF CORRECTION**

PATENT NO. : 6,214,133 B1  
DATED : April 10, 2001  
INVENTOR(S) : Seetharama C. Deevi et al.

Page 1 of 2

It is certified that error appears in the above-identified patent and that said Letters Patent is hereby corrected as shown below:

Title page.

**ABSTRACT**, line 1, delete "titanic" and insert therefor -- titanium --;

Column 1.

Line 25, delete "668673" and insert therefor -- 668-673 --;

Line 30, delete "Cr and S" and insert therefor -- Cr and Si --;

Column 2.

Line 8, delete "tansus" and insert therefor -- transus --;

Line 9, delete "% laths" and insert therefor --  $\alpha_2$  laths --;

Line 13, between lines 13 and 14 should be inserted -- SUMMARY OF THE INVENTION --;

Column 3.

Line 4, delete "PMTAL" and insert therefor -- PMTA-6 --;

Line 56, delete "TiAl alloys" and insert therefor -- TiAl alloys --;

Column 5.

Line 3, delete "PMTAA" and insert therefor -- PMTA-4 --;

Column 6.

Line 54, delete "TiAl alloys" and insert therefor -- TiAl alloys --;

Line 58, delete "PMTA 14" and insert therefor -- PMTA 1-4 --;

Line 62, delete "TiAlCr" and insert therefor -- TiAlCr --;

Line 63, delete "TiAlCr" and insert therefor -- TiAlCr --;

Line 65, delete "PMTAA" and insert therefor -- PMTA-4 --;

Column 8.

Line 8, delete " $\rho_{uc}$ " and insert therefor --  $\sigma_{uc}$  ---;

Column 9.

Line 48, delete "MoSs" and insert therefor -- MoSi<sub>2</sub> --; and

UNITED STATES PATENT AND TRADEMARK OFFICE  
**CERTIFICATE OF CORRECTION**

PATENT NO. : 6,214,133 B1  
DATED : April 10, 2001  
INVENTOR(S) : Seetharama C. Deevi et al.

Page 2 of 2

It is certified that error appears in the above-identified patent and that said Letters Patent is hereby corrected as shown below:

Column 10.

Line 7, delete "Mu-free" and insert therefor -- Mn-free --;

Signed and Sealed this

Twenty-third Day of April, 2002

Attest:

Attesting Officer

JAMES E. ROGAN  
Director of the United States Patent and Trademark Office

